

## UNITED STATES PATENT OFFICE

FRANK B. ROOT, OF EAST ORANGE, NEW JERSEY, ASSIGNOR TO CHADELOID CHEMICAL COMPANY, OF NEW YORK, N. Y., A CORPORATION OF VIRGINIA

## RUGOUS COATING COMPOSITION AND PROCESS OF MAKING SAME

No Drawing.

Application filed November 20, 1929. Serial No. 408,662.

This invention relates to a liquid coating composition containing a binder preferably of the cellulose ester type, such as nitrocellulose or acetyl cellulose, and also containing ground wood or wood flour, preferably of spray-projecting fineness, coatings formed by the application of spraying of such composition preferably having the property of drying rapidly at room temperature to form a textured rugous surface.

The vehicle of the coating composition as stated is preferably of the cellulose ester type such, for example, as a solution in appropriate solvents of low viscosity nitrocellulose, a plasticizer and a resin. A lacquer vehicle of this character forms the carrier for the ground wood material essential in forming the textured rugous surface. Instead of using lacquers or similar rapidly drying compositions, I may in some cases employ a quick drying oil varnish. When the latter is used the acceleration of drying by mild baking is not precluded. Likewise, if desired, baking may be resorted to in the case of the cellulose lacquer, but baking involves an additional step with loss of time and labor expense and I preferably, as indicated, employ a very rapid drying vehicle in order that the textured surface may be produced in the quickest possible time at a minimum of labor cost.

Ground wood or wood flour varies in particle size, some being quite coarse and others very fine. The ground wood obtained from soft woods such as poplar, pine, spruce, fir, and the like, which is ordinarily employed as a filler in molding compositions, linoleum, and the like, may be used in carrying out the present invention. Also it is possible to employ ground wood prepared from hard woods. Cedar dust likewise may be employed in some cases.

In the preferred form of the invention it is an object to employ the ground wood in a state of palpability or coarseness adequate to secure a textured surface of a decidedly

rugous character but, on the other hand, of a particle size not exceeding spray-projecting fineness, since I preferably apply my composition by means of a spray-gun. The latter implement has become thoroughly standard- 50 ized and its orifices and connecting tubes are of such character that coarse particles will not pass therethrough. I have found, however, particles of ground wood of soft wood origin seemingly of a size which would clog 55 the spray nozzles will pass through these relatively tiny orifices and be projected in the spray upon the surface which is to be coated, forming a rugous coating of a decorative textured character.

There is, however, a limit to the fineness of the ground wood which I prefer to employ, since the use of ground wood in the form of an impalpable powder tends to give merely a dull surface of a non-rugous character. 65 While I do not avoid the employment of ground wood containing a percentage of tiny particles which, if separated, would yield an impalpable powder, nevertheless I find it highly advantageous to employ a screened 70 mixture of the ground wood from which the impalpable particles have been removed, likewise the coarse particles of spray-clogging dimensions. In this way I secure a texture-producing ingredient of spray-project- 75 ing fineness largely free from impalpable wood powder. In other words, I prefer to employ ground wood in the form of a palpable powder largely free from impalpa- 80 ble material.

The wood flour of soft wood origin preferably is entirely free from bark or dirt in discoloring proportion in order that the coating may be pigmented by colors, lakes or pig- 85 ments, or the wood flour itself dyed to yield, when desired, coatings of desirable tone or tint. In some cases the wood flour may be dyed and the vehicle itself may carry another color with the object of securing some con- 90

trast between the rugous wood particles of the coating and the binder.

Another possible decorative effect is that secured by spraying the composition on surfaces which are held vertically and allowing a certain slippage or downward movement to take place resulting in slight separations into ridgelike formations or elevated areas intermediate which is an area occupied by the vehicle alone perhaps dotted with a few particles of the ground wood; such effect being to give a more emphatic texture to the surface, which oftentimes is desirable. The formations, or sliprugae, obtained in this manner serve as demarcation or aggregation areas which viewed from a distance of a few feet afford to the eye a textured appearance of high decorative value. In this manner I may treat the interior walls of buildings to form textured surfaces. For example, the composition may be applied to plaster which has been well sized and after the spray coating has dried the textured effect described will be found well developed.

Such a textured surface oftentimes may be improved in vigor or depth by applying a coating of a clear composition such as clear lacquer or varnish, preferably the former. The second coat or supercoat may be tinted in any desired manner by colors, lakes, pigments, and so forth.

A further feature of my invention is the proportioning of ground wood to binder. In a lacquer vehicle composed of nitrocellulose, plasticizer, resin and solvents in about normal proportions, I find a proportion of about one part of wood flour of said spray-projecting fineness to two parts of solid contents of the vehicle is suitable. This ratio varies somewhat with the different kinds of wood particles. It may be as high as one part of wood flour to one part of vehicle solids in certain cases.

The following will serve to illustrate my invention:

*Example 1*

| Per cent |                           |
|----------|---------------------------|
| 6.6      | 1/2 second nitrocellulose |
| 5.4      | ester gum                 |
| 50 2     | dibutyl phthalate         |
| 30       | ethyl acetate             |
| 2        | ethyl alcohol             |
| 22       | butyl acetate             |
| 25       | toluol                    |
| 65 7     | spruce flour              |

This mixture constitutes a coating composition of good spray-projecting qualities and gives a finish of desirable texture. The mixture is of such viscosity that the wood flour settles very slowly and after it has settled it can easily be redispersed by shaking or stirring. Instead of ester gum in the above composition I may use any natural or synthetic resin that is compatible with nitrocellulose. Also, instead of dibutyl phthalate

I may use any suitable plasticizer, such as castor oil, tricresyl phosphate, alkyl ether of a polyglycol, and so forth. I prefer to use nitrocellulose of low viscosity since wood flour naturally produces a viscous mixture. The use of high viscosity nitrocellulose would tend to give too viscous a mixture for application. In this respect the resins and plasticizers are of value in giving high solid content of the vehicle without increasing the viscosity very much.

I prefer to use a wood flour the particles of which have a substantially definite size. In the above example the flour was passed through a 30 mesh screen and the larger particles discarded, these being of spray-clogging size. The smaller particles were then removed by means of a 120 mesh screen and these were discarded. That is, the flour was of such particle size that all passed through a 30 mesh screen but was retained by a 120 mesh screen.

If desired the more impalpable particles may not be separated. However, since they do not assist in the attainment of a textured surface and absorb a certain portion of the vehicle, I prefer to separate them as described.

I may use any wood flour of soft wood origin. Also, I may use a wood flour of hard wood origin, such as oak, gum, maple, and so forth. If the spruce flour in the above example is replaced by the same amount of hard wood flour, there is less absorption of the binder by the flour and a coating having more gloss is obtained. To get the same dullness of surface using a hardwood flour, the proportion of the latter must be increased. Thus in Example 1, I may use as much as 14 per cent of hardwood flour and obtain a spray-projecting composition which produces a highly desirable textured quality when applied. To avoid the disadvantage of the greater settling of hardwood flour due to its higher density, I may use a mixture of two or more forms of wood flour.

A particular advantage of the composition designated Example 1 is its film-building ability. On a vertical surface a film can be built up in one application the thickness of which greatly exceeds that which is possible with the ordinary sprayed coating. The ordinary sprayed coating runs off a vertical surface if a very heavy film is applied, but with the composition here described a quite heavy coat is permissible. Another advantage of this type of composition is its very great covering power. For example, one coat applied to a piece of bare wood produces a uniform color which completely hides the grain configuration of the wood underneath.

If a very heavy film of the composition designated Example 1 is applied to a vertical, more or less impervious surface, some downward sliding of the film occurs producing

5 segregated ridges bounded by substantially smooth areas. The formation of slip-rugae as described above is facilitated by lower viscosity of the mixture. For example, if I add 5 an extra 20 per cent of a solvent mixture to Example 1 and spray a heavy coat on a vertical surface, there is a very noticeable formation of irregular ridges or slip-rugae which produces a very desirable texture-contrast.

10 *Example 2*

| Per cent |                           |
|----------|---------------------------|
| 6        | 1/2 second nitrocellulose |
| 3        | ester gum                 |
| 2        | dibutyl phthalate         |
| 15       | 25 ethyl acetate          |
| 28       | butyl acetate             |
| 2        | butyl alcohol             |
| 26       | 26 toluol                 |
| 20       | 8 ground vegetable ivory  |

25 The above mixture forms a composition of good spray-projecting qualities and produces a dull gray textured coating. The coating is more glossy than Example 1. This is due 25 to the harder quality of vegetable ivory, that is, it does not absorb so much of the vehicle as wood flour does. Vegetable ivory being denser than wood flour settles a little faster but it can readily be redispersed by shaking 30 or stirring the mixture. The ground vegetable ivory was passed through a 30 mesh screen and the larger particles of spray-clogging dimensions were discarded. Ground vegetable ivory contains a certain amount of 35 brown particles due to the shell. This is not objectionable if a pigment is used in the lacquer to modify the color.

40 Since vegetable ivory is of greater density than wood flour and therefore has a greater 40 tendency to settle out of the mixture, it is well to use a mixture of wood flour and vegetable ivory. Thus I may use a mixture consisting of equal parts of wood flour and ground vegetable ivory. This mixture 45 settles much more slowly than the vegetable ivory alone. Also the composition containing this mixture has very desirable spray-projecting qualities.

50 *Example 3*

| Per cent |                           |
|----------|---------------------------|
| 5        | 1/2 second nitrocellulose |
| 3        | dammar                    |
| 1        | castor oil                |
| 55       | 1 dibutyl phthalate       |
| 30       | ethyl acetate             |
| 2        | ethyl alcohol             |
| 22       | butyl acetate             |
| 30       | 20 toluol                 |
| 60       | 6 cedar dust              |

65 This mixture is of very desirable spray-projecting consistency and when sprayed it produces by means of one coat a rich brown textured coating without the use of a pigment. However, a pigment may be used if

desired to modify the color. The cedar dust used in this example was passed through a 30 mesh screen and all the larger particles were discarded. The more or less impalpable particles may or may not be removed. A certain percentage of these particles is desirable for their tinting qualities, although they are of no advantage in producing the textured effect.

70 By use of this composition it is possible 75 to obtain a finish on bare wood or sized plaster, or other more or less rigid surfaces, by one coat due to the high covering (hiding) power of the cedar dust.

80 *Example 4*

| Per cent |                           |
|----------|---------------------------|
| 6        | 1/2 second nitrocellulose |
| 2        | castor oil                |
| 1        | dibutyl phthalate         |
| 30       | ethyl acetate             |
| 2        | ethyl alcohol             |
| 24       | butyl acetate             |
| 30       | 26 toluol                 |
| 5        | 5 cork dust               |

90 This composition is also of excellent spray-projecting character and produces a dark brown textured coating without the use of any pigment. The cork dust which I used was of the commercial grade used in the linoleum industry. It was screened to 30 mesh size without separating the more impalpable particles.

95 *Example 5*

| Per cent |                           |
|----------|---------------------------|
| 5        | 1/2 second nitrocellulose |
| 4        | rosin ester               |
| 1        | dibutyl phthalate         |
| 30       | ethyl acetate             |
| 2        | ethyl alcohol             |
| 18       | butyl acetate             |
| 30       | 26 toluol                 |
| 6        | wood flour                |
| 4        | 4 gold bronze             |

100 This is a mixture of good spray-projecting qualities and produces a textured finish which is a combination of the effects given by the other examples and that of the gold bronze.

105 Clipped hair, shredded asbestos, mineral wool, cotton linters, cotton flock and silk flock, when used alone are much more difficult to convert to spray-projecting comminution. Mixed with a lacquer the fibres normally tend to mat together somewhat so that the mixture cannot be as readily applied by spray-gun or brush. However, used in admixture with a palpable material of the requisite spray-projecting type they greatly assist the latter in forming a textured surface. Thus I 115 may use 20 per cent of finely shredded asbestos and 80 per cent of wood flour in a lacquer, as set forth above, and obtain a composition 120 of good texturing qualities.

125 In any of the above examples I may add a 130

coloring agent such as pigment or dye to give any desired shade. Thus in Example 1, I may add Prussian blue, say 4 per cent, and produce a blue texturing material which gives the desired color and textured coating by means of one coat. That is, I may give bare wood or other surfaces a textured and suitably colored coating in one application.

I may also use the compositions listed above 10 as undercoats over which to apply a coating of lacquer enamel, varnish enamel, clear shellac or any other clear coating composition.

For example, the composition designated 15 Example 1, may be applied to a surface and dried, giving a rough textured coating. This rough coating is then sprayed with a lacquer, for example, the following:

| Per cent |                        |
|----------|------------------------|
| 20       | 6 ----- nitrocellulose |
|          | 3 ----- ester gum      |
|          | 8 ----- gold bronze    |
|          | 83 ----- thinner       |

The applied lacquer is thus used to give the 25 colored effect upon the rough textured surface which is an undercoat.

In the foregoing I have indicated the possibility when treating vertical surfaces to secure slip-rugae. This result, however, can 30 be secured only when a thin solution is used of adequate sagging properties. Under normal conditions the lacquer containing the ground wood or similar material can be applied as a coat of a fairly uniform character 35 so far as concealing or hiding power is concerned. A very surprising result is obtained by using the product of the present invention as a one-coat finish in that complete coverage and hiding of the under surface is obtained 40 by the application of a single coat. In the ordinary nitrocellulose lacquer pigmentation, especially in the lighter shades, cannot be carried to such a degree that a single coat will properly conceal or hide the under surface 45 face. In the present invention by the employment of wood fibres and the like, acting somewhat similar to blotting paper, I am able to build up by a single sprayed application a one-coat finish which provides full concealment of the surface without dripping of the 50 lacquer vehicle. I therefore disclose the process of application which comprises spraying a lacquer containing a drip-arrester whereby a covered surface adapted as a complete finish is secured in a single coat. In 55 other words, a one-coat rugous sprayed finish completely concealing the surface beneath results.

What I claim is:

60 1. A liquid coating composition containing palpable ground wood of substantially soft wood origin and of spray-projecting fineness; said coating composition rapidly drying on exposure at room temperature to form 65 a textured rugous surface.

2. A liquid coating composition containing palpable ground wood of substantially soft wood origin and of spray-projecting fineness; said coating composition rapidly drying on exposure at room temperature on a vertical 70 surface to form a textured finish containing slip-rugae.

3. A decorative nitrocellulose wall lacquer containing palpable ground wood of soft wood origin and of spray-projecting fineness; said lacquer drying to a rugous surface. 75

4. A decorative wall lacquer containing palpable ground wood of soft wood origin and of spray-projecting fineness; said lacquer drying to a rugous surface. 80

5. An article of manufacture carrying a finish of a rugous character containing ground wood of spray-projecting fineness held in position by a binding agent and super-coated with a lacquer. 85

6. A rugous drying lacquer carrying as a pigment cedar sawdust of between 20 and 120 mesh.

7. A rugous drying lacquer carrying as a pigment cedar sawdust not exceeding about 90 20 mesh.

8. A rugous drying lacquer carrying as a pigment cedar sawdust not exceeding spray-delivering coarseness.

9. In a one-coat spraying lacquer a texture-forming agent comprising a non-caking free-spraying component of pulverized wood. 95

10. The process which consists in screening pulverized wood to remove chips and coarse particles and then incorporating the screened product in a nitrocellulose lacquer of low viscosity in proportion to give a spray-projecting coating composition capable of forming in one application a rugous coating adequate to completely conceal the supporting surface. 105

11. Rugous-forming lacquer finishes containing low viscosity nitrocellulose and palpable ground wood of spray-projecting fineness. 110

12. Rugous-forming lacquers containing a cellulose pigment.

13. An article of manufacture carrying a rugous film adherent thereto, said film comprising a fibrous rugosifier of spray-delivering fineness and a binding agent. 115

14. An article of manufacture carrying a rugous film adherent thereto, said film comprising a cellulose fibre rugosifier of spray-delivering fineness and a binding agent. 120

FRANK B. ROOT.